

## UNITED STATES PATENT OFFICE

BERTRAND W. STORY, OF WOODBURY, NEW JERSEY, ASSIGNOR TO VACUUM OIL COMPANY, INC., OF NEW YORK, N. Y., A CORPORATION OF NEW YORK

## TRANSFORMER OIL

No Drawing.

Application filed March 31, 1926. Serial No. 98,921.

The present invention relates to transformer oils and an object thereof is to provide an oil having improved property with respect to the formation of insoluble sludge. 3 when subjected to oxidation, without introducing at the same time other properties of an undesirable nature such as poor electrical characteristics, affinity for moisture and high vapor pressure. 10 Transformer oils, as made by properly refining certain petroleum fractions, gradually oxidize in service and, in those types of transformer oil to which my invention relates, there occurs ultimately a formation of insoluble sludge. This precipitation of sludge is highly objectionable since it is usually less soluble in cool oil than in hot oil and precipitates in the cooling ducts of the transformer. Being a good insulator the sludge prevents the oil from giving up its heat causing the temperature of the transformer to rise beyond safe working limits. When sludge precipitates from oil in a transformer it is customary practice to remove the 15 oil for reconditioning or replacement by new oil; a matter of considerable trouble and expense.

In order to retard the sludging tendency of said transformer oils, it has been proposed to introduce therein glycerine. This suggestion has been found, however, of little practical value, due to the fact that the use of glycerine in transformer oils causes other effects of an undesirable nature, as for instance, a reduction of dielectric strength and specific resistance.

I have discovered that the sludging tendency of transformer oils can be retarded, without introducing, at the same time, undesirable properties, such as affinity for moisture and high vapor pressure, by introducing an alcohol having substantial anti-oxidizing qualities, combined with a relatively low vapor pressure and affinity for water. The material which I have found most available for this purpose is cetyl alcohol.

In illustration of my invention, I will describe the retarding effect on the sludging tendency of a transformer oil as determined 10 in the life test for transformer oils (A. S. T.

M., report of committee D-9, page 17; publications of American Society for Testing Materials, Philadelphia, Penna.), brought about by the addition of cetyl alcohol



53

to said transformer oil.

A transformer oil, having a specific gravity of 0.9 and a viscosity of 55 seconds at 104° F. gave a life test of 16 days when tested according to the method specified above. The addition of one-tenth of one percent by weight of cetyl alcohol increased the life test of said transformer oil to 26 days; while the addition of five-tenths of one percent of cetyl alcohol increased the life test of said transformer oil to 50 days.

60

Any alcohol, such as glycerine, having a high affinity for moisture will necessarily impair the dielectric strength and specific resistance of an oil into which it is introduced. Alcohols having a carbon-atom content of more than seven are relatively nonhygroscopic. To this fact the value of cetyl alcohol may be largely attributed, and other alcohols of high carbon-atom content may be expected to have similarly valuable qualities, though not now commercially available for the use in question.

70

While, in the above illustration of my invention, I have described the desirable effects of certain proportions of cetyl alcohol when added to a given transformer oil, I wish it understood that I do not limit myself to any specific proportions of this alcohol or 75 of any other alcohol coming within the scope of my invention.

80

What I claim as my invention and desire to secure by Letters Patent is:

A petroleum transformer oil having added 90 thereto cetyl alcohol.

BERTRAND W. STORY.

95

100